

Nov. 11, 1958

D. J. WEST ET AL

2,860,078

HEAT TREATMENT FOR TITANIUM BASE ALLOY, CIRCA 4% Mn, AND 4% Al

Filed May 25, 1955



INVENTORS.  
DONALD J. WEST  
RICHARD A. BAUGHMAN  
BY

*Lee H. Jacobs*

ATTORNEY-

# United States Patent Office

2,860,078

Patented Nov. 11, 1958

1

2,860,078

## HEAT TREATMENT FOR TITANIUM BASE ALLOY, CIRCA 4% Mn, AND 4% Al

Donald John West and Richard Augustus Baughman,  
Cincinnati, Ohio, assignors to General Electric Company,  
a corporation of New York

Application May 25, 1955, Serial No. 511,114

6 Claims. (Cl. 148—13)

This invention relates to a process for heat treating titanium and in particular to a process for heat treating a particular type of titanium alloy in order to make it ductile.

Compressor wheels on a turbojet engine are a critical part of the engine and are subjected to high migratory 20 stresses when rotating at high velocity. Also, large stress concentrations take place when the turbojet engine undergoes sudden bursts of thrust during transient operation. The points of stress concentrations take place in areas where there is a tendency for the stresses to build up. If the material undergoing these stress concentrations has ductility, the material can undergo plastic deformation at the point of stress concentration and relieve the stress. If the stress concentration continues to build up and is not relieved, it can result in the form of an initial fracture which will later destroy the part and perhaps destroy the engine. This problem becomes particularly critical during the high temperatures and speeds of a jet engine at which time the velocity of rotating parts is also exceedingly high, so that any initial fracture will be seriously aggravated and undoubtedly do a lot of damage to the engine. Since titanium alloy has a good strength weight ratio, the use of compressor wheels made from titanium alloys is very desirable in order to achieve considerable weight savings in the engine. However, one of the undesirable features of titanium is that it tends to remain brittle mainly because of the impurities contained in the alloy itself or becomes brittle when subjected to the high temperatures. Therefore, the ductility necessary to meet the specification requirements is a problem confronting the entire titanium industry. It is therefore a general object of this invention to provide a process for heat treating titanium articles to give them the necessary ductility during engine operating conditions regardless of temperature and speed.

In forging titanium, the article is formed high in the beta and alpha plus beta range to give the material the necessary ductility. However, in forming articles in the beta and alpha plus beta range, it has been difficult to consistently obtain the ductility properties that are required by specifications, thereby resulting in large amounts of scrapped titanium articles. The reported literature is deficient in data relating to heat treating cycles to produce a material ductile and stable enough to allow the manufacture of titanium alloy articles. Since titanium is a very expensive material, scrapping becomes a very expensive loss. In general, approximately 50 percent of the compressor wheels made of titanium and heat treated to previous processes, fail to meet the required specifications for ductility and are rejected. It is therefore another object of this invention to provide a process for heat treating titanium articles to consistently meet the required specification for ductility.

It is an object of this invention to provide a process for isothermally heat treating a titanium alloy at various

2

temperatures in the beta or alpha plus beta phases and slowly furnace cooling the alloy at another temperature in the alpha plus beta phase without permitting the formation of fine alpha structure thereby obtaining improved ductility.

It is another object of this invention to heat treat a titanium alloy consisting of approximately 4 percent manganese, 4 percent aluminum and the rest titanium and its impurities so as to impart to that alloy the necessary 10 ductility to meet the required specifications by stabilizing the alloy against age hardening, embrittlement and build-up of stresses at temperatures up to about 800° F.

These and other objects will become more apparent when read in the light of the accompanying specification taken in connection with the attached drawing. The scope of my invention will be pointed out in the appended claims.

In general, the invention may be practiced by heating an alloy comprising about 4% manganese, about 4% aluminum with the balance essentially titanium to a temperature just within the beta range, the area marked "beta" in the drawing, or high in the range in which only coarse alpha will form, shown by the shaded portion in the drawing, maintaining the alloy at this temperature 25 for a period of time, transforming the alloy isothermally to a lower temperature in the range in which only coarse alpha will form, and then transforming the alloy to at least one temperature in the alpha plus beta range by cooling it slowly, and lastly cooling to room temperature.

30 The isothermal heat treating process herein described is similar to that disclosed in co-pending patent application, Serial No. 511,115, filed May 25, 1955, and assigned to the present assignee of this application. The process differs however, in that the alloy as therein described may be initially heated to a temperature high 35 within the range in which only coarse alpha will form to create as much beta structure as possible instead of heating the alloy completely to the beta phase. If the process taught by the above-mentioned co-pending application is used with the alloy as herein described, a structure will result which is not as ductile as that resulting from the heat treatment disclosed by this application.

In order to heat treat titanium alloy articles made of approximately 4 percent manganese, 4 percent aluminum and the rest titanium and its impurities, so as to have the necessary ductility to meet the required specification, the first step is to betatize the article by heating it to approximately 1720° F. into the area marked "beta" on the drawing. Betatizing is heat treating the alloy in

50 the beta field, and we maintain it as low as possible in the beta field so as to form a beta structure with a minimum amount of alpha phase before transforming into the alpha plus beta field. This stabilizing temperature is maintained for approximately 50 minutes. By 55 staying at the low temperature in the beta field, the material in general will contain beta structure before transforming back into the alpha plus beta structure at the lower temperature.

60 The next step in the process is the isothermal heat treating portion in which the material is cooled to approximately 1380° F. into the area between the shaded portion and the beta+alpha regions of the drawing by transferring it to another furnace which perhaps is already 65 at the 1380° F. temperature or staying in the furnace and cooling it down to the 1380° F. temperature. At the 1380° F. temperature coarse alpha is allowed to form. However, if a sufficiently lower temperature than 1380° F. is used, fine alpha structure will be formed. It is noted 70 that the fine alpha structure in the material causes the brittleness to occur when cooling down to room temper-

ature. It is further noted that if the material is held at a higher temperature than the 1380° F. temperature, less alpha will form in reaching the equilibrium condition so that upon subsequent cooling more fine alpha will be formed thereby causing brittleness. The stabilizing time has been found to be approximately 75 minutes. This is a minimum time and is critical in order to maintain an isothermal condition until equilibrium between alpha and the beta phases is established.

After stabilizing the material at 1380° F., the material is then cooled to 1300° F. within the beta+alpha region of the drawing for stabilizing at this temperature. This step is necessary since after cooling from the 1380° F. temperature additional alpha may be formed. In other words, at any lower temperature, more alpha is present at equilibrium conditions than at the 1300° F. or 1380° F. temperatures. The beta to alpha transformation is a time temperature phenomenon. In order to have alpha and beta in equilibrium at a given temperature, sufficient time for transformation must be allowed. Also, the lower the temperature, the slower the reaction. Therefore, longer times are required for the 1300° F. temperature than for the 1380° F. to allow the alpha and beta phases to reach an equilibrium condition and prevent the formation of an unstable beta phase upon subsequent cooling to room temperature. If insufficient time is allowed at the 1300° F. temperature, and unstable beta forms, then a fine precipitate will form from the unstable beta during subsequent engine operation, thereby causing the loss of ductility of the part. It is therefore necessary to stabilize the material at the 1300° F. temperature for a minimum of two hours.

The next step of the process is to cool the alloy to another temperature in the alpha plus beta range which in this instance is approximately 900° F. It is not necessary to isothermally heat treat the material at this temperature, but merely to furnace cool from the 1300° F. temperature to the 900° F. temperature at a slow rate. The material becomes stabilized as it transforms from the 1300° F. temperature to the 900° F. temperature.

The last step of the process is to cool the material to room temperature by taking the article out of the furnace. It is noted that cooling down to room temperature by taking the article out of the furnace is much better than to furnace cool since brittleness may result because of furnace cooling thereby making the ductility of the material low.

Another embodiment of the invention has been found in heat treating this titanium alloy to a high temperature in the alpha beta field without going into the beta field so as to form a large percentage of beta, holding this temperature for a considerable period of time and then furnace cooling to a lower temperature in the alpha plus beta field, and holding this temperature to stabilize the structure, and then furnace cooling to a still lower temperature in the alpha beta field after which the material is air cooled to room temperature. More specifically, the alloy is heated to approximately 1600° F. for a period of eight hours in order to insure that the material has been stabilized. This stabilizing time is longer than the above referred to method so as to form sufficient beta. In other words, the stabilizing time is longer. The next step is to furnace cool to 1300° F. and maintain it at this temperature for a period of two hours. The next step is then to furnace cool to 900° F. at a slow rate from the 1300° F. temperature to the 900° F. temperature. It is not necessary to stabilize upon reaching the 900° F. temperature. After having reached the 900° F. temperature, the material is then air cooled to room temperature.

The following table which is a summary of tests conducted on seven different heats of material compares the physical properties of the titanium base alloy containing about 4% manganese and about 4% aluminum before and after our novel heat treatment.

The marked increase in ductility is especially to be noted:

|                             | Before  | After   |
|-----------------------------|---------|---------|
| Tensile Strength (p. s. i.) | 153,400 | 151,200 |
| Percent Elongation (in 1")  | 10.4    | 15.2    |
| Percent Reduction in Area   | 15.7    | 24.7    |

10 In order to show the stability of this particular type of titanium alloy after our novel heat treatment process, a series of compressor wheel forgings were aged for up to about 1000 hours. The following table summarizes the results of aging showing the uniform increased ductility.

|    | Aging Temp. (° F.) | Hours at Temp. | Tensile Strength (p. s. i.) | Percent Elongation (in 1") |
|----|--------------------|----------------|-----------------------------|----------------------------|
| 20 | 700                | 0              | 151                         | 17                         |
|    | 700                | 110            | 150                         | 19                         |
|    | 700                | 265            | 152                         | 18                         |
|    | 700                | 405            | 154                         | 15                         |
|    | 700                | 600            | 156                         | 16                         |
| 25 | 700                | 1,100          | 156                         | 16                         |

Therefore, in order to prevent titanium alloy materials from becoming brittle upon being subjected to relatively high temperatures when in use, the alloy has been heat treated isothermally and stabilized at various temperatures in the beta and alpha plus beta range in order to prevent fine alpha structure from being formed either during the heat treat process or upon being subjected to the high temperatures when being used.

35 The above example of the invention has been given by way of illustration and is not intended as a limitation of the invention. The times and temperatures given can vary within narrow limits according to the characteristics of the material since it may contain various percentages of impurities or the like. However, such variations are intended to be included within the spirit and scope of this invention since they are regarded as equivalents.

What we claim as new and desired to secure by Letters Patent of the United States is:

1. The process of heat treating a titanium alloy including about 4% manganese and about 4% aluminum comprising heat treating the material to the lowest temperature in the beta range at approximately 1720° F. to form the beta phase and maintaining this temperature until such time as the material becomes betatized, cooling the material to 1380° F. and maintaining this temperature for approximately 75 minutes permitting coarse alpha phase in equilibrium with beta phase to form without permitting fine alpha structure to form, cooling the alloy to 1300° F. and maintaining this temperature for approximately 120 minutes to prevent fine alpha from forming, slowly furnace cooling from 1300° F. to 900° F. to prevent fine alpha from forming, and then air cooling from about 900° F. to room temperature.

2. In a heat treating process for a titanium alloy including about 4% manganese and about 4% aluminum comprising heating the alloy to a temperature in the beta range for a sufficient length of time until the material becomes betatized, cooling to a temperature in the range in which only coarse alpha will form and holding this temperature for a sufficient amount of time to permit coarse alpha to form, cooling to a first temperature in the alpha plus beta range and stabilizing the material for a period of time to prevent age hardening, slowly furnace cooling from the first temperature in the alpha plus beta range to a second temperature in the alpha plus beta range to prevent fine alpha from forming, and air cooling this material from the second temperature in the alpha plus beta range to room temperature.

3. In a heat treating process for a titanium alloy including about 4% manganese and about 4% aluminum, com-

prising heating the alloy to a first temperature in a phase in which only coarse alpha can form but sufficiently high to form beta phase, maintaining this temperature for a sufficient length of time to stabilize the material, cooling to a second temperature in the range in which only coarse alpha can form and maintaining this temperature for a sufficient length of time to permit the material to become stabilized, furnace cooling slowly from the last temperature to a temperature in the alpha plus beta range, and then air cooling the material from the temperature in the alpha plus beta range to room temperature.

4. In the process for heat treating a titanium alloy including about 4% manganese and about 4% aluminum comprising heat treating the alloy to 1600° F. for eight hours to permit the material to become stabilized, cooling to 1300° F. and maintaining this temperature for two hours to permit the material to become stabilized, slowly furnace cooling from 1300° F. to 900° F. to prevent fine alpha structure from forming in the material, and air cooling from 900° F. to room temperature.

5. In a process for heat treating an alloy consisting of 4 percent manganese, 4 percent aluminum and the remainder titanium and its impurities comprising heat treating the alloy to 1600° F. for a sufficient length of time for

the material to become stabilized, cooling to 1300° F. for a sufficient length of time for the material to become stabilized, slowly furnace cooling from 1300° F. to 900° F., and air cooling from 900° F. to room temperature.

5 6. In a process for heat treating an alloy consisting of 4 percent manganese, 4 percent aluminum and the remainder titanium and its impurities comprising heat treating the alloy to 1720° F. for a sufficient length of time until the material becomes betatized, cooling the alloy to 1380° F. for a sufficient length of time for the material to become stabilized, cooling the alloy to 1300° F. for a sufficient length of time for the material to become stabilized, slowly furnace cooling the alloy to 900° F., and air cooling the alloy from 900° F. to room temperature.

15

References Cited in the file of this patent

UNITED STATES PATENTS

|           |                     |               |
|-----------|---------------------|---------------|
| 2,596,485 | Jaffee et al. ----- | May 13, 1952  |
| 2,754,203 | Vordahl -----       | July 10, 1956 |

20

OTHER REFERENCES

Atlas of Isothermal Transformations, U. S. Steel, pages 6-26, 1951.